

May 8, 1956

G. R. RADLEY

2,744,839

COATED ELECTRICAL APPARATUS AND METHOD OF MAKING THE SAME

Filed Aug. 24, 1953

Fig. 1



Fig. 2



Fig. 3



Fig. 4



Fig. 5



Fig. 6



Fig. 7



Inventor  
Guy R. Radley  
By *W. Shipp*  
Attorney

2,744,839

**COATED ELECTRICAL APPARATUS AND METHOD OF MAKING THE SAME**

Guy R. Radley, Whitefish Bay, Wis., assignor to Cutler-Hammer, Inc., Milwaukee, Wis., a corporation of Delaware

Application August 24, 1953, Serial No. 376,039

4 Claims. (Cl. 117—218)

This invention relates to improved methods of and means for protecting electrical apparatus from moisture and mechanical damage.

While not limited thereto, the invention is especially useful for protecting electrical windings and terminal connectors of electrical apparatus.

A primary object of the invention is to provide improved methods and means for protecting electrical apparatus against mechanical damage and the harmful effects of moisture.

Another object is to provide, for electrical apparatus, improved coatings which have long life, are resistant to mechanical abrasion, and are impervious to moisture.

Another object is to provide coatings of the aforescribed character which readily dissipate heat.

Another object is to provide improved wire-wound electrical resistors having protective coatings which will readily dissipate heat and will afford, for the resistance windings and for the connections between the windings and the resistor terminals, increased protection against corrosion and mechanical damage.

Various other objects and advantages of the invention will hereinafter appear.

The accompanying drawings illustrate certain embodiments of the invention and the steps of producing the same, which will now be described, it being understood that other embodiments are possible without departing from the spirit or scope of the invention as defined in the appended claims.

In the drawings, Figure 1 is an elevational view of an electrical resistor unit which is representative of one of the classes of electrical apparatus to which the invention is applicable;

Fig. 2 is an enlarged, fragmentary, sectional view illustrating one step in the production of a coating embodying the invention as applied to a resistor unit;

Fig. 3 is an enlarged, fragmentary, sectional view illustrating a part of a resistor unit provided with a protective coating embodying the invention;

Fig. 4 is an enlarged, fragmentary, sectional view illustrating one step in the production of a coating of alternative form embodying the invention as applied to a resistor unit;

Fig. 5 is an enlarged, fragmentary, sectional view illustrating a part of a resistor unit provided with a protective coating of alternative form embodying the invention;

Fig. 6 is an elevational view of a resistor unit provided with a coating embodying the invention; and

Fig. 7 is an enlarged, fragmentary, view of a part of a resistor unit showing a preferred method of connecting resistance wire to an end terminal.

In addition to being made safe and shock-proof, certain types of electrical apparatus must be protected against corrosion, electrolytic action, mechanical vibration, abrasion and the like. Of these types, certain ones have

high operating temperatures and are required to dissipate substantial amounts of heat. While not limited thereto, this invention is particularly useful in protecting apparatus of the latter type. Because wire-wound resistors are subjected to the most severe of these conditions, the application of the invention to such resistors will be described, it being understood that the application and usefulness of the invention is not limited thereto.

A representative form of wire-wound resistor is shown 10 in Fig. 1. It consists of an insulating base 10, a length of resistance wire 12 coiled thereabout and a pair of ferrule-like end connector members 14 and 16. Each end of wire 12 is fastened to one of a pair of short pieces 13, 13 of wire which are tucked under a respectively associated one of the end connector members 14 and 16. The connector members or terminals are clamped or spun against the base 10 and said pieces of wire 13 so that they have good electrical contact with the latter. In normal use the uncoated resistance wire 12 expands 20 and may become loose enough to permit adjacent turns of the wire to touch one another. Merely coating the unit with an adhesive material is not an adequate remedy, for if such material is of sufficiently low viscosity for uniform application thereof, its surface tension will cause 25 it to flow away from the upper surfaces of the wire. Such upper surfaces will thereafter be unprotected against abrasion and other mechanical damage and, if touched, may result in serious electrical shock. Also, if the coating becomes crazed, moisture will be admitted and will 30 corrode the wire and may form an electrolyte with certain chemical constituents of the base 10 or of the coating and effect electrolytic action between the turns of the resistance wire and also between the resistance wire and the end connector members 14 and 16. The aforescribed difficulties and others are overcome by applicant's invention in which the apparatus to be protected is first provided with a layer 18 (Fig. 2) of a mixture of adhesive material 20 and solid filler material 22. The adhesive material is then hardened. A second layer 40 24 of adhesive material is applied over the first layer (see Fig. 3) and is hardened.

The filler material 22 in the first layer 18 of adhesive material gives "body" to said layer to permit its even application to the apparatus to be protected by spraying, 45 brushing, or dipping methods and so that the effect of surface tension is substantially overcome. Wires, such as wire 12, and the like, are substantially covered by adhesive and filler material. After the adhesive material is hardened, the filler material acts to inhibit crazing of the 50 layer.

Protection of the apparatus against moisture and protection of the coating against heat is afforded by the use of waterproof and heat resistant adhesive and filler materials. I prefer to employ a resinous adhesive material 55 such as silicone resin and a filler comprising grains of quartz. Approximately equal volumes of Dow Corning number 802 silicone resin and Dow Corning number 803 silicone resin, to which is added enough solvent such as toluol so that the resulting mixture has a specific gravity about equal to that of water, provide a satisfactory liquid adhesive mixture. When from one-fourth to two-thirds of a part of quartz grains about one mil in diameter are added to one part of the liquid, the resulting mixture is one which may be applied to articles by dipping, brushing, 60 or spraying methods.

This layer is then air dried until a "skin" forms on the outer surface. The drying time depends largely upon the composition of the adhesive material. Usually drying for about one hour is sufficient. The layer is then baked to hardness beginning at a low temperature. The 65 temperature is increased gradually or may be increased 70

in steps over a period of hours. The maximum temperature is usually that which the base material can withstand without warping or blistering or otherwise being damaged. It is desirable that the final baking temperature be about 500° Fahrenheit when the characteristics of the base material permit.

The resulting layer is very strong and tough and will not craze at temperatures as high as 700° F. The space between the resistance wires is substantially filled. However, the surface may be somewhat rough and certain portions of the resistance wire may not be sufficiently covered. A second layer 24 of adhesive material, preferably comprising the same material as the first layer 18 but not including filler material, is applied over said first layer. A coloring agent or coloring matter may be mixed with the second layer of adhesive 24 before it is applied to improve the heat dissipating qualities of the protective coating. Dark colors are preferred. Black is best because it radiates heat at a greater rate than other colors so that the resistor can be given a higher watt rating when its coating is colored black. The addition of powdered magnetic iron oxide to the adhesive material will color the mixture black. This material will retain its color, even when subjected to the maximum safe operating temperature of resistors, and has good dielectric strength.

The second layer 24 is then hardened in the same manner as was the first layer 18. The resultant coating has a pebbled outer surface which withstands higher operating temperatures than does a smooth surface composed of the same materials. This coating has unusually good heat dissipation characteristics, a very tough, hard, waterproof and heat resistant inner layer and a relatively less hard outer layer having expansion characteristics like that of the inner layer. The resinous adhesive material adheres tenaciously to the base material and to the wires so that the protective coating is not lifted away from the base by expansion of the wire.

In certain instances, as where the resistance wire 12 is of large diameter, it is desirable to sprinkle or otherwise apply larger particles 26 of filler material (see Fig. 4) on the first layer of adhesive material 20 and filler material 22 before said first layer is air dried or baked. The larger particles 26 of filler material are permitted to embed themselves in the adhesive material 20 and may be further covered by the application of additional quantities of the mixture of adhesive material 20 and small grains of filler material 22. The resultant layer 28 is then air dried and baked in the manner aforescribed. As shown in Fig. 5, a second layer 30 of adhesive material, which may be mixed with coloring matter, is then applied over layer 28 and is air dried and baked.

The large particles of filler material 26 are preferably egg-shaped and have smooth surfaces so that the upper surface of layer 28, while pebbled, is relatively smooth, and so that layer 30 will be of relatively uniform thickness. I now prefer to employ particles, ranging in size from about 5 to 10 mils diameter, of a sand which comprises quartz and zircon. Such sand is found along portions of the shores of the Gulf of Mexico and is commercially available under the trade name "Zircon."

A resistor of the type illustrated in Fig. 1, to which a protective coating 32 has been applied, is illustrated in Fig. 6. The protective coating 32 extends partly over the end connector members or terminals 14 and 16 of the resistor so that the points at which the resistance

wire is tucked under and connects to the respective terminals are completely covered. Thus entry of moisture at said points and subsequent electrolytic action between the wire and the terminals which would result in oxidation of the resistance wire and, consequently, poor electrical connections between the wire and terminals, is prevented. Because of the protection against moisture which is afforded by the coating, it is possible to connect the resistance wire to the resistor terminals without soldering, welding or other expensive and troublesome procedures. As illustrated in detail in Fig. 7, a short length of wire 13, preferably of the same metal as the resistance wire 12, is firmly clamped between the terminal 14 and the base 10 by the process known as "spinning." The end of the resistance wire 12 is twisted with the short wire 13 and the twisted connection is thereafter bent down against the base 10. The protective coating is applied over the twisted joint and over the "spun" end of ferrule 14 to protect the twisted joint from deterioration.

I claim:

1. In producing a protective coating on electrical apparatus, the steps of applying a mixture comprising one part of liquid silicone resin adhesive material and from one-fourth to two-thirds of a part of particles of heat resistant mineral filler material having a diameter of about one mil, to the surface to be protected, embedding particles of substantially smooth surfaced heat resistant mineral filler material having a diameter of approximately five to ten mils in the mixture of adhesive material and particles of filler material, air drying and baking said adhesive material to harden the same, applying a second layer comprising a mixture of liquid silicone resin adhesive material and dark coloring matter over the first layer of filler materials and hardened adhesive, and thereafter air drying and heating said second layer to harden the same.

2. The subject matter of claim 1 wherein the dark coloring matter is black and of good dielectric strength.

3. An article comprising electrical apparatus having thereon a protective coating consisting of a first layer comprising a mixture of one part of hardened silicone resin and from one-fourth to two-thirds of a part of particles of heat resistant mineral filler material and having particles of approximately five to ten mils diameter of substantially smooth surfaced and heat resistant mineral filler material embedded therein, and a second layer bonded to said first layer and comprising a mixture of hardened silicone resin and coloring matter.

4. The subject matter of claim 3 wherein the coloring matter is black and of good dielectric strength.

#### References Cited in the file of this patent

#### UNITED STATES PATENTS

|           |                |                |
|-----------|----------------|----------------|
| 2,093,501 | Williams       | Sept. 21, 1937 |
| 2,229,985 | Nowak et al.   | Jan. 28, 1941  |
| 2,258,218 | Rochow         | Oct. 7, 1941   |
| 2,290,905 | Butler         | July 28, 1942  |
| 2,330,365 | Jackson        | Sept. 28, 1943 |
| 2,459,018 | DeMonte et al. | Jan. 11, 1949  |
| 2,523,037 | Mathes         | Sept. 19, 1950 |
| 2,523,065 | Sage           | Sept. 19, 1950 |
| 2,531,169 | Sprung         | Nov. 21, 1950  |
| 2,664,364 | Thom           | Dec. 29, 1953  |